

## UNITED STATES PATENT OFFICE

2,246,288

## DENTAL ALLOY

Maude Braid, Hartsdale, N. Y.

No Drawing. Application July 2, 1940,  
Serial No. 343,559

2 Claims. (CL 75—171)

This invention relates to an alloy of the class containing nickel and chromium and more particularly relates to an alloy suitable for dental purposes, i. e. for dentures, plates, pins, etc. as well as other purposes in which high resistance to corrosive attack is an essential.

An object of my invention is to provide an improved alloy particularly suitable for dental purposes.

A further object of the invention is to provide an improved alloy possessing a tensile strength and hardness greater than that of the ordinary nickel-chrome alloys and one which while ductile has its yield point sufficiently high for use as a denture.

A further object of the invention is to provide an improved dental alloy which is malleable, forgeable and entirely workable for denture use while having a high resistance to corrosive attack.

With these and other objects in view the invention consists in an alloy comprising as its essential ingredients chromium, nickel, cobalt, molybdenum, tungsten and zirconium.

In this alloy the chromium, nickel and cobalt are the usual and natural elements for denture use. The molybdenum acts to lower the melting point and increase the fluidity while the tungsten is employed for its toughening and hardening qualities. I regard the inclusion of zirconium as a novel and essential ingredient in this type of alloy. It has a two-fold advantage firstly as a hardener but more importantly as a powerful deoxidizer.

The ingredients of my new alloy may be employed in a wide range of percentages, for example—

|            | Per cent<br>by weight |
|------------|-----------------------|
| Chromium   | 10—49                 |
| Nickel     | 10—40                 |
| Cobalt     | 20—48                 |
| Molybdenum | 3—15                  |
| Tungsten   | 3—12                  |
| Zirconium  | .25—3                 |

but I have found that for use as a denture the following composition is to be preferred viz:

|              | Per cent<br>by weight |
|--------------|-----------------------|
| 5 Chromium   | 30                    |
| Nickel       | 15                    |
| Cobalt       | 45                    |
| Molybdenum   | 5                     |
| Tungsten     | 5                     |
| 10 Zirconium | .25                   |

In the production of my new alloy I prefer to employ the relatively recently known process of alloying known as "powder metallurgy" which briefly stated consists in fine grinding the metals, e. g. to 250 mesh, intimately mixing the same and placing the mixture in a die in which it is subjected to high pressure (of the order of 50 tons). A hard solid mass results which is then inserted into a furnace and subjected to sintering heat. It will be noted that at no time are the metals melted.

This process is particularly advantageous in the production of my new alloy as by it I am enabled to control very closely the proportions of each ingredient in the final product as losses particularly of molybdenum and zirconium due to volatilization are avoided or greatly minimized. It will be understood however that I do not confine myself to using this process of production of the alloy as any usual or known process may equally well be employed.

What I claim is:

1. An alloy consisting of 10—49% chromium, 20—48% cobalt, 3—15% molybdenum, 10—40% nickel, 3—12% tungsten and 0.25—3% zirconium.
2. An alloy consisting of about 30% chromium, about 45% cobalt, about 15% nickel, about 5% molybdenum, about 5% tungsten and about 0.25% zirconium.

MAUDE BRAID.